



US010961477B2

(12) **United States Patent**  
**Ali et al.**

(10) **Patent No.:** **US 10,961,477 B2**  
(b5) **Date of Patent:** **\*Mar. 30, 2021**

(54) **FUEL ADDITIVES**(71) Applicant: **BP OIL INTERNATIONAL LIMITED**, Sunbury on Thames (GB)(72) Inventors: **Rana Ali**, Reading (GB); **Sorin Vasile Filip**, Reading (GB)(73) Assignee: **BP OIL INTERNATIONAL LIMITED**, Sunbury On Thames (GB)

(\*) Notice: Subject to any disclaimer, the term of this patent is extended or adjusted under 35 U.S.C. 154(b) by 0 days.

This patent is subject to a terminal disclaimer.

(21) Appl. No.: **16/077,459**(22) PCT Filed: **Feb. 9, 2017**(86) PCT No.: **PCT/EP2017/052933**

§ 371 (c)(1),

(2) Date: **Aug. 11, 2018**(87) PCT Pub. No.: **WO2017/137521**PCT Pub. Date: **Aug. 17, 2017**(65) **Prior Publication Data**

US 2019/0071613 A1 Mar. 7, 2019

(30) **Foreign Application Priority Data**

Feb. 11, 2016 (EP) ..... 16155212

(51) **Int. Cl.**  
**C10L 1/23** (2006.01)  
**C10L 1/233** (2006.01)  
(Continued)(52) **U.S. Cl.**  
CPC ..... **C10L 1/2335** (2013.01); **C10L 1/023** (2013.01); **C10L 1/233** (2013.01); **C10L 10/10** (2013.01);  
(Continued)(58) **Field of Classification Search**CPC ..... C10L 1/2335; C10L 10/10; C10L 1/233; C10L 1/023; C10L 2200/0423; C10L 2270/023; C10L 2290/24; C10L 2290/141  
See application file for complete search history.(56) **References Cited**

## U.S. PATENT DOCUMENTS

1,833,429 A 11/1931 Lovell et al.  
2,560,898 A 7/1951 Schulze et al.  
(Continued)

## FOREIGN PATENT DOCUMENTS

CN 101389738 A 3/2009  
CN 101451080A A 6/2009  
(Continued)

## OTHER PUBLICATIONS

Han, Jeong Sik et al., "Liquid fuel composition with improved thermal stability", Dec. 2012, XP002759592, retrieved from STN, Database accession No. 2012:1371756.

(Continued)

Primary Examiner — Cephia D Toomer

(74) Attorney, Agent, or Firm — McDonnell Boehnen Hulbert &amp; Berghoff LLP

(57) **ABSTRACT**

An additive composition for use in a fuel for a spark-ignition internal combustion engine comprises an octane-boosting additive and one or more further fuel additives. The octane-boosting additive has a chemical structure comprising a 6-membered aromatic ring sharing two adjacent aromatic carbon atoms with a 6- or 7-membered saturated heterocyclic ring, the 6- or 7-membered saturated heterocyclic ring comprising a nitrogen atom directly bonded to one of the shared carbon atoms to form a secondary amine and an atom selected from oxygen or nitrogen directly bonded to the other shared carbon atom, the remaining atoms in the 6- or 7-membered heterocyclic ring being carbon. The additive

(Continued)

composition increases the octane number of the fuel, thereby proving the auto-ignition characteristics of a fuel.

|    |             |    |        |
|----|-------------|----|--------|
| WO | 2010/01341  | A2 | 1/2010 |
| WO | 2012/120147 | A1 | 9/2012 |
| WO | 2015/003961 | A1 | 1/2015 |

### 18 Claims, 4 Drawing Sheets

- (51) **Int. Cl.**  
*C10L 10/10* (2006.01)  
*C10L 1/02* (2006.01)
- (52) **U.S. Cl.**  
CPC . *C10L 2200/0423* (2013.01); *C10L 2270/023* (2013.01); *C10L 2290/141* (2013.01); *C10L 2290/24* (2013.01)

### (56) References Cited

#### U.S. PATENT DOCUMENTS

|                  |         |                  |
|------------------|---------|------------------|
| 2,881,061 A      | 4/1959  | Brennan et al.   |
| 2,948,600 A      | 8/1960  | Larson           |
| 4,304,712 A      | 12/1981 | Lai              |
| 4,421,522 A      | 12/1983 | Seemuth          |
| 4,552,672 A      | 11/1985 | Walker           |
| 7,976,591 B2     | 7/2011  | Paggi et al.     |
| 8,016,898 B1     | 9/2011  | Lange et al.     |
| 8,409,474 B2     | 4/2013  | Lange et al.     |
| 9,017,429 B2     | 4/2015  | Griffiths et al. |
| 9,217,115 B2     | 12/2015 | Lange et al.     |
| 2004/0021637 A1  | 2/2004  | Ahn              |
| 2009/0107555 A1* | 4/2009  | Aradi .....      |
|                  |         | C10L 1/14        |
|                  |         | 137/13           |

#### FOREIGN PATENT DOCUMENTS

|    |                |         |
|----|----------------|---------|
| CN | 102234549 A    | 11/2011 |
| CN | 105085504 A    | 11/2015 |
| DE | 2926183 A1     | 1/1980  |
| EP | 0234753 A1     | 9/1987  |
| GB | 2308849 *      | 7/1997  |
| JP | 2003511491 A   | 3/2003  |
| JP | 2009502857 A   | 1/2009  |
| KR | 101297655 B1   | 8/2013  |
| WO | 2001053436 A1  | 7/2001  |
| WO | 2005/087901 A2 | 9/2005  |

#### OTHER PUBLICATIONS

- Mizar P et al., "Synthesis of substituted 4-(3-alkyl-1,2,4-oxadiazol-5-ylmethyl)-3,4-dihydro-2H-1,4-benzoxazines and 4-(1H-benzimidazol-2-ylmethyl)-3,4-dihydro-2H-1,4-benzoxazines", *Tetrahedron Letters*, 47(44): 7823-7826, Oct. 30, 2006.
- Goudert, "A new synthesis of 3,4-dihydro-2H-1,4-benzoxalines using solid-liquid phase transfer catalysis", *Communications*, pp. 541-543, Jul. 1, 1979.
- Fu et al., "Simple and efficient synthesis of novel n-dichloroacetyl-3,4-dihydro-2H-1,4-benzoxazines", Dec. 2012, XP002759652, Database accession No. 2014:557179.
- Mizar P et al., "Synthesis of 2,3-dihydro-6H-1-oxa-3a-azaphenalene and its benzolhetero-fused analog", *Journal of Heterocyclic Chemistry*, 48(5): 1187-1191, May 5, 2011.
- Inoue T et al., "Carboxylic acid compound having URAT1 activity-inhibitory effect, and use thereof", Dec. 2007, XP002759595, retrieved from STN, Database accession No. 2007:841279.
- Perry B et al., "Achieving multi-isoform PI3K inhibition in a series of substituted 3,4-dihydro-2Hbenzo[1,4]oxazines", *Bioorganic & Medicinal Chemistry Letters*, 18(16):4700-4704, Aug. 15, 2008, XP002759654, Database accession No. 2008:960774.
- Dominczak N et al., "A very short and efficient palladiumcatalyzed access to the 3,4-dihydro-2H-1,4-benzoxazine structure", *Letters in Organic Chemistry*, 3(5), 371-373, 2006, XP002759655, retrieved from STN, Database accession No. 2006:623620.
- Liu Z et al., "Efficient synthesis of 2,3-dihydro-1,4-benzoxazines via intramolecular copper-catalyzed 0-arylation", *Tetrahedron Letters*, 50(27): 3790-3793, Jul. 8, 2009.
- International Search Report and Written Opinion of the International Search Authority for International Application No. PCT/EP20171052933, dated Apr. 7, 2017.
- Search Report for EP 16155212.0, dated Jul. 22, 2016.
- Park et al. "Mechanistic Insights into Thermal Stability Improvement of exo-Tetrahydronyclopentadiene by a New Hydrogen Donor." *Energy & Fuels*, 2015, vol. 29, No. 1, pp. 16-20.
- Park et al. "Thermal Stability Improvement of exo-Tetrahydronyclopentadiene by 1,2,3,4-Tetrahydroquinoxaline." *J. Phys. Chem. C*, 2013, vol. 117, No. 15, 7399-7497.

\* cited by examiner

Fig. 1a



Fig. 1b



Fig. 1c



Fig. 2a



Fig. 2b



Fig. 2c



# 1

## FUEL ADDITIVES

This application is a national stage application under 35 U.S.C. § 371 of International Application No. PCT/EP2017/052933, filed Feb. 9, 2017, which claims priority to European Patent Application No. EP 16155212.0, filed Feb. 11, 2016, the disclosures of which are explicitly incorporated by reference herein.

### FIELD OF THE INVENTION

This invention relates to additive compositions for use in a fuel for a spark-ignition internal combustion engine. In particular, the invention relates to additive compositions comprising octane-boosting additives for use in increasing the octane number of a fuel for a spark-ignition internal combustion engine. The invention further relates to containers and kits comprising octane-boosting additives.

### BACKGROUND OF THE INVENTION

Spark-ignition internal combustion engines are widely used for power, both domestically and in industry. For instance, spark-ignition internal combustion engines are commonly used to power vehicles, such as passenger cars, in the automotive industry.

Combustion in spark-ignition internal combustion engines is initiated by a spark which creates a flame front. The flame front progresses from the spark-plug and travels across the combustion chamber rapidly and smoothly until almost all of the fuel is consumed.

Spark-ignition internal combustion engines are widely thought to be more efficient when operating at higher compression ratios, i.e. when a higher degree of compression is placed upon the fuel/air mix in the engine prior to its ignition. Thus, modern, high performance spark-ignition internal combustion engines tend to operate at high compression ratios. Higher compression ratios are also desired when an engine has a high degree of supplemental pressure boosting to the intake charge.

However, increasing the compression ratio in an engine increases the possibility of abnormal combustion including that of auto-ignition, particularly when the engine is pressure-boosted. A form of auto-ignition occurs when the end gas, typically understood to be the unburnt gas between the flame front and combustion chamber walls/piston, ignites spontaneously. On ignition, the end gas burns rapidly and prematurely ahead of the flame front in the combustion chamber, causing the pressure in the cylinder to rise sharply. This creates the characteristic knocking or pinking sound and is known as “knock”, “detonation” or “pinking”. In some cases, particularly with pressure-boosted engines, other forms of auto-ignition can even lead to destructive events known as “mega-knock” or “super-knock”.

Knock occurs because the octane number (also known as the anti-knock rating or the octane rating) of the fuel is below the anti-knock requirement of the engine. Octane number is a standard measure used to assess the point at which knock will occur for a given fuel. A higher octane number means that a fuel/air mixture can withstand more compression before auto-ignition of the end gas occurs. In other words, the higher the octane number, the better the anti-knock properties of a fuel. Whilst the research octane number (RON) or the motor octane number (MON) may be used to assess the anti-knock performance of a fuel, in recent

# 2

literature more weight is being given to the RON as an indicator of a fuel's anti-knock performance in modern automotive engines.

Accordingly, there is a need for fuels for spark-ignition internal combustion engines which have a high octane number, e.g. a high RON. There is a particular need for fuels for high compression ratio engines, including those utilising a high degree of supplemental pressure boosting to the intake charge, to have a high octane number so that higher engine efficiency may be enjoyed in the absence of knock.

In order to increase the octane number, octane improving additives are typically added to a fuel. Such additisation may be carried out by refineries or other suppliers, e.g. fuel terminals or bulk fuel blenders, so that the fuel meets applicable fuel specifications when the base fuel octane number is otherwise too low.

Organometallic compounds, comprising e.g. iron, lead or manganese are well-known octane improvers, with tetraethyl lead (TEL) having been extensively used as a highly effective octane improver. However, TEL and other organometallic compounds are generally now only used in fuels in small amounts, if at all, as they can be toxic, damaging to the engine and damaging to the environment.

Octane improvers which are not based on metals include oxygenates (e.g. ethers and alcohols) and aromatic amines. However, these additives also suffer from various drawbacks. For instance, N-methyl aniline (NMA), an aromatic amine, must be used at a relatively high treat rate (1.5 to 2% weight additive/weight base fuel) to have a significant effect on the octane number of the fuel. NMA can also be toxic. Oxygenates give a reduction in energy density in the fuel and, as with NMA, have to be added at high treat rates, potentially causing compatibility problems with fuel storage, fuel lines, seals and other engine components.

Effort has been made to find alternative non-metallic octane improvers to NMA. GB 2 308 849 discloses dihydro benzoxazine derivatives for use as anti-knock agents. However, the derivatives provide a significantly smaller increase in the RON of a fuel than is provided by NMA at similar treat rates.

Accordingly, there remains a need for additives for a fuel for a spark-ignition internal combustion engine that are able to achieve anti-knock effects, e.g. at least comparable anti-knock effects to NMA, while mitigating at least some of the problems highlighted above.

### SUMMARY OF THE INVENTION

Surprisingly, it has now been found that an additive having a chemical structure comprising a 6-membered aromatic ring sharing two adjacent aromatic carbon atoms with a 6- or 7-membered saturated heterocyclic ring, the 6- or 7-membered saturated heterocyclic ring comprising a nitrogen atom directly bonded to one of the shared carbon atoms to form a secondary amine and an atom selected from oxygen or nitrogen directly bonded to the other shared carbon atom, the remaining atoms in the 6- or 7-membered heterocyclic ring being carbon, provides a substantial increase to the octane number, particularly the RON, of a fuel for a spark-ignition internal combustion engine. Such octane-boosting additives are also predicted to exhibit lower toxicity than NMA. Reduced toxicity would enable additive compositions, containers and kits comprising the octane-boosting additives to provide octane-boosting benefits, whilst being easily stored, transported, used and disposed of.

Accordingly, the present invention provides an additive composition for use in a fuel for a spark-ignition internal

combustion engine, the additive composition comprising an octane-boosting additive having a chemical structure comprising a 6-membered aromatic ring sharing two adjacent aromatic carbon atoms with a 6- or 7-membered saturated heterocyclic ring, the 6- or 7-membered saturated heterocyclic ring comprising a nitrogen atom directly bonded to one of the shared carbon atoms to form a secondary amine and an atom selected from oxygen or nitrogen directly bonded to the other shared carbon atom, the remaining atoms in the 6- or 7-membered heterocyclic ring being carbon, and one or more further fuel additives.

The present invention also provides a container comprising:

- (i) an octane-boosting additive described herein; and
- (ii) means configured to introduce the octane-boosting additive into a fuel system.

The present invention further provides a container comprising an octane-boosting additive in an amount which is: (a) suitable for treating a fuel in a fuel tank or a fuel tanker at a rate of 0.1% to 10%, more preferably from 0.2% to 5%, still more preferably from 0.25% to 2%, and even more preferably still from 0.3% to 1% weight additive/weight base fuel;

(b) suitable for increasing the octane number of a fuel in a fuel tank or a fuel tanker by at least 0.5, preferably at least 1, more preferably at least 2, and still more preferably at least 2.5; or

(c) greater than 100 ml, preferably greater than 150 ml, and more preferably greater than 200 ml;

wherein the octane-boosting additive is as described herein.

Also provided is a kit comprising:

an octane-boosting additive described herein; and instructions for using the octane-boosting additive in a fuel for a spark-ignition internal-combustion engine.

The octane-boosting additive described herein preferably has the formula:



where: R<sub>1</sub> is hydrogen;

R<sub>2</sub>, R<sub>3</sub>, R<sub>4</sub>, R<sub>5</sub>, R<sub>11</sub> and R<sub>12</sub> are each independently selected from hydrogen, alkyl, alkoxy, alkoxy-alkyl, secondary amine and tertiary amine groups;

R<sub>6</sub>, R<sub>7</sub>, R<sub>8</sub> and R<sub>9</sub> are each independently selected from hydrogen, alkyl, alkoxy, alkoxy-alkyl, secondary amine and tertiary amine groups;

X is selected from —O— or —NR<sub>10</sub>—, where R<sub>10</sub> is selected from hydrogen and alkyl groups; and n is 0 or 1.

Other aspects of the present invention include the use of an additive composition described herein in a fuel for a spark-ignition internal-combustion engine, and the use of an additive composition described herein for increasing the octane number of a fuel for a spark-ignition internal combustion engine, as well as for improving the auto-ignition characteristics of a fuel, e.g. by reducing the propensity of the fuel for at least one of auto-ignition, pre-ignition, knock, mega-knock and super-knock, when used in a spark-ignition internal combustion engine.

Also provided is a method for increasing the octane number of a fuel for a spark-ignition internal combustion engine, as well as a method for improving the auto-ignition characteristics of a fuel, e.g. by reducing the propensity of a fuel for at least one of auto-ignition, pre-ignition, knock, mega-knock and super-knock, when used in a spark-ignition internal combustion engine, said methods comprising blending an additive composition described herein with the fuel.

A fuel composition comprising an additive composition described herein is also provided.

#### BRIEF DESCRIPTION OF THE FIGURES

FIGS. 1a-c show graphs of the change in octane number (both RON and MON) of fuels when treated with varying amounts of an octane-boosting additive described herein. Specifically, FIG. 1a shows a graph of the change in octane number of an E0 fuel having a RON prior to additisation of 90; FIG. 1b shows a graph of the change in octane number of an E0 fuel having a RON prior to additisation of 95; and FIG. 1c shows a graph of the change in octane number of an E10 fuel having a RON prior to additisation of 95.

FIGS. 2a-c show graphs comparing the change in octane number (both RON and MON) of fuels when treated with octane-boosting additives described herein and N-methyl aniline. Specifically, FIG. 2a shows a graph of the change in octane number of an E0 and an E10 fuel against treat rate; FIG. 2b shows a graph of the change in octane number of an E0 fuel at a treat rate of 0.67% w/w; and FIG. 2c shows a graph of the change in octane number of an E10 fuel at a treat rate of 0.67% w/w.

#### DETAILED DESCRIPTION OF THE INVENTION

##### Octane-Boosting Additive

The present invention provides additive compositions, kits, containers, uses and methods in which an octane-boosting additive is used.

The octane-boosting additive has a chemical structure comprising a 6-membered aromatic ring sharing two adjacent aromatic carbon atoms with a 6- or 7-membered otherwise saturated heterocyclic ring, the 6- or 7-membered saturated heterocyclic ring comprising a nitrogen atom directly bonded to one of the shared carbon atoms to form a secondary amine and an atom selected from oxygen or nitrogen directly bonded to the other shared carbon atom, the remaining atoms in the 6- or 7-membered heterocyclic ring being carbon (referred to in short as an octane-boosting additive described herein). As will be appreciated, the 6- or 7-membered heterocyclic ring sharing two adjacent aromatic carbon atoms with the 6-membered aromatic ring may be considered saturated but for those two shared carbon atoms, and may thus be termed “otherwise saturated.”

Alternatively stated, the octane-boosting additive used in the present invention may be a substituted or unsubstituted 3,4-dihydro-2H-benzo[b][1,4]oxazine (also known as benzomorpholine), or a substituted or unsubstituted 2,3,4,5-tetrahydro-1,5-benzoxazepine. In other words, the additive may be 3,4-dihydro-2H-benzo[b][1,4]oxazine or a derivative thereof, or 2,3,4,5-tetrahydro-1,5-benzoxazepine or a derivative thereof. Accordingly, the additive may comprise one or more substituents and is not particularly limited in relation to the number or identity of such substituents.

Preferred additives have the following formula:



where: R<sub>1</sub> is hydrogen;

R<sub>2</sub>, R<sub>3</sub>, R<sub>4</sub>, R<sub>5</sub>, R<sub>11</sub> and R<sub>12</sub> are each independently selected from hydrogen, alkyl, alkoxy, alkoxy-alkyl, secondary amine and tertiary amine groups;

R<sub>6</sub>, R<sub>7</sub>, R<sub>8</sub> and R<sub>9</sub> are each independently selected from hydrogen, alkyl, alkoxy, alkoxy-alkyl, secondary amine and tertiary amine groups;

X is selected from —O— or —NR<sub>10</sub>—, where R<sub>10</sub> is selected from hydrogen and alkyl groups; and n is 0 or 1.

In some embodiments, R<sub>2</sub>, R<sub>3</sub>, R<sub>4</sub>, R<sub>5</sub>, R<sub>11</sub> and R<sub>12</sub> are each independently selected from hydrogen and alkyl groups, and preferably from hydrogen, methyl, ethyl, propyl and butyl groups. More preferably, R<sub>2</sub>, R<sub>3</sub>, R<sub>4</sub>, R<sub>5</sub>, R<sub>11</sub> and R<sub>12</sub> are each independently selected from hydrogen, methyl and ethyl, and even more preferably from hydrogen and methyl.

In some embodiments, R<sub>6</sub>, R<sub>7</sub>, R<sub>8</sub> and R<sub>9</sub> are each independently selected from hydrogen, alkyl and alkoxy groups, and preferably from hydrogen, methyl, ethyl, propyl, butyl, methoxy, ethoxy and propoxy groups. More preferably, R<sub>6</sub>, R<sub>7</sub>, R<sub>8</sub> and R<sub>9</sub> are each independently selected from hydrogen, methyl, ethyl and methoxy, and even more preferably from hydrogen, methyl and methoxy.

Advantageously, at least one of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub>, and preferably at least one of R<sub>6</sub>, R<sub>7</sub>, R<sub>8</sub> and R<sub>9</sub>, is selected from a group other than hydrogen. More preferably, at least one of R<sub>7</sub> and R<sub>8</sub> is selected from a group other than hydrogen. Alternatively stated, the octane-boosting additive may be substituted in at least one of the positions represented by R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub>, preferably in at least one of the positions represented by R<sub>6</sub>, R<sub>7</sub>, R<sub>8</sub> and R<sub>9</sub>, and more preferably in at least one of the positions represented by R<sub>7</sub> and R<sub>8</sub>. It is believed that the presence of at least one group other than hydrogen may improve the solubility of the octane-boosting additives in a fuel.

Also advantageously, no more than five, preferably no more than three, and more preferably no more than two, of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> are selected from a group other than hydrogen. Preferably, one or two of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> are selected from a group other than hydrogen. In some embodiments, only one of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> is selected from a group other than hydrogen.

It is also preferred that at least one of R<sub>2</sub> and R<sub>3</sub> is hydrogen, and more preferred that both of R<sub>2</sub> and R<sub>3</sub> are hydrogen.

In preferred embodiments, at least one of R<sub>4</sub>, R<sub>5</sub>, R<sub>7</sub> and R<sub>8</sub> is selected from methyl, ethyl, propyl and butyl groups and the remainder of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> are hydrogen. More preferably, at least one of R<sub>7</sub> and R<sub>8</sub> are selected from methyl, ethyl, propyl and butyl groups and the remainder of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> are hydrogen.

In further preferred embodiments, at least one of R<sub>4</sub>, R<sub>5</sub>, R<sub>7</sub> and R<sub>8</sub> is a methyl group and the remainder of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> are hydrogen. More preferably, at least one of R<sub>7</sub> and R<sub>8</sub> is a methyl group and the remainder of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> are hydrogen.

Preferably, X is —O— or —NR<sub>10</sub>—, where R<sub>10</sub> is selected from hydrogen, methyl, ethyl, propyl and butyl groups, and preferably from hydrogen, methyl and ethyl groups. More preferably, R<sub>10</sub> is hydrogen. In preferred embodiments, X is —O—.

n may be 0 or 1, though it is preferred that n is 0.

Octane-boosting additives that may be used in the present invention include:



Preferred octane-boosting additives include:



A mixture of additives may be used. For instance, a mixture of:



may be used in the present invention.

It will be appreciated that references to alkyl groups include different isomers of the alkyl group. For instance, references to propyl groups embrace n-propyl and i-propyl groups, and references to butyl embrace n-butyl, isobutyl, sec-butyl and tert-butyl groups.

#### Additive Composition

In aspects of the present invention, the octane-boosting additives described herein may be used in an additive composition which comprises one or more further fuel additives.

The octane-boosting additive may be present in the additive composition in an amount of at least 10% by weight, preferably from 15% to 95% by weight, more preferably from 20% to 80% by weight, and still more preferably from 30% to 80% by weight of the additive composition.

Examples of further fuel additives that may be present in the additive compositions include detergents, friction modifiers/anti-wear additives, corrosion inhibitors, combustion modifiers, anti-oxidants, valve seat recession additives, dehazers/demulsifiers, dyes, markers, odorants, anti-static agents, anti-microbial agents, and lubricity improvers. Preferably, at least one of the one or more further fuel additives is a detergent.

Further octane improvers may also be used in the additive composition, i.e. octane improvers which are not octane-boosting additives described herein, i.e. they do not have a chemical structure comprising a 6-membered aromatic ring sharing two adjacent aromatic carbon atoms with a 6- or 7-membered saturated heterocyclic ring, the 6- or 7-membered saturated heterocyclic ring comprising a nitrogen atom directly bonded to one of the shared carbon atoms to form a secondary amine and an atom selected from oxygen or nitrogen directly bonded to the other shared carbon atom, the remaining atoms in the 6- or 7-membered heterocyclic ring being carbon.

Examples of suitable detergents include polyisobutylene amines (PIB amines) and polyether amines.

Examples of suitable friction modifiers and anti-wear additives include those that are ash-producing additives or ashless additives. Examples of friction modifiers and anti-wear additives include esters (e.g. glycerol mono-oleate) and fatty acids (e.g. oleic acid and stearic acid).

Examples of suitable corrosion inhibitors include ammonium salts of organic carboxylic acids, amines and heterocyclic aromatics, e.g. alkylamines, imidazolines and tolyl-triazoles.

Examples of suitable anti-oxidants include phenolic anti-oxidants (e.g. 2,4-di-tert-butylphenol and 3,5-di-tert-butyl-4-hydroxyphenylpropionic acid) and aminic anti-oxidants (e.g. para-phenylenediamine, dicyclohexylamine and derivatives thereof).

Examples of suitable valve seat recession additives include inorganic salts of potassium or phosphorus.

Examples of suitable further octane improvers include non-metallic octane improvers include N-methyl aniline and nitrogen-based ashless octane improvers. Metal-containing octane improvers, including methylcyclopentadienyl manganese tricarbonyl, ferrocene and tetra-ethyl lead, may also be used. However, in preferred embodiments, the additive composition is free of all added metallic octane improvers including methylcyclopentadienyl manganese tricarbonyl and other metallic octane improvers including e.g. ferrocene and tetraethyl lead.

Examples of suitable dehazers/demulsifiers include phenolic resins, esters, polyamines, sulfonates or alcohols which are grafted onto polyethylene or polypropylene glycols.

Examples of suitable markers and dyes include azo or anthraquinone derivatives.

Examples of suitable anti-static agents include fuel soluble chromium metals, polymeric sulfur and nitrogen compounds, quaternary ammonium salts or complex organic alcohols. However, the additive composition is preferably substantially free from all polymeric sulfur and all metallic additives, including chromium based compounds.

In some embodiments, the additive composition comprises solvent, e.g. which has been used to ensure that the additives are in a form in which they can be stored or combined with the liquid fuel. Examples of suitable solvents include polyethers and aromatic and/or aliphatic hydrocarbons, e.g. heavy naphtha e.g. Solvesso (Trade mark), xylenes and kerosene.

#### Containers and Kits

In an aspect of the invention, a container comprises an octane-boosting additive described herein, and means configured to introduce the octane-boosting additive into a fuel system.

In embodiments, the means configured to introduce the octane-boosting additive into a fuel system are replaceable, e.g. the means may be removed and reattached to the container in a non-destructive manner, and/or a replacement means may be attached to the container in a non-destructive manner. "A non-destructive manner" will be understood as meaning that integrity of the container is largely unaltered, aside from the possible breakage and/or destruction of disposable elements of the container.

In other embodiments, the means configured to introduce the octane-boosting additive into a fuel system form an integral part of the container, and cannot be replaced, e.g. the means may not be removed or reattached in a non-destructive manner.

In preferred embodiments, the means are configured to couple the container to the fuel system. Coupling is intended to describe mechanical interactions between the means and the fuel system, e.g. screw and thread and click-locking systems, as well as interference fit systems in which a force is imparted from a resilient member (e.g. a resilient member which forms part of the coupling means may impart a force onto the fuel system, or vice versa). The means may com-

prise a male part which is configured to couple to a female part in the fuel system. Alternatively, the means may comprise a female part which is configured to couple to a male part in the fuel system.

In other embodiments, the means configured to introduce the octane-boosting additive into the fuel system do not couple with the fuel system. In these embodiments, the means may comprise a male part which is simply inserted into a female part in the fuel system. Alternatively, the means may comprise a female part designed to receive a male part from the fuel system.

In preferred embodiments, the means configured to introduce the octane-boosting additive into a fuel system comprise at least one of a spout, a funnel and an injector.

The means and/or fuel system may further comprise a seal. A seal serves to prevent the octane-boosting additive described herein from spilling during its introduction into a fuel system.

The fuel system may comprise an engine, or a fuel tanker.

The engine preferably forms part of a vehicle, preferably an automotive vehicle such as a motorcycle or a passenger car, though static engines are also anticipated. The engine may comprise pipework and a fuel tank which stores fuel for combustion in a chamber in the engine.

The fuel system may be a fuel tanker which is transported on a vehicle, such as a lorry. However, the fuel tanker may also be a static tanker, such as a fuel storage tanker.

In another aspect of the invention, a container, e.g. a container as described previously, comprises an octane-boosting additive described herein in an amount which is suitable for treating a base fuel in a fuel tank or a fuel tanker at a rate of up to 20%, preferably from 0.1% to 10%, more preferably from 0.2% to 5%, still more preferably from 0.25% to 2%, and even more preferably still from 0.3% to 1% weight additive/weight base fuel. It will be appreciated that, when more than one octane-boosting additive described herein is used, these values refer to the total amount of octane-boosting additive described herein in the fuel.

Alternatively or additionally, the container, e.g. a container as described previously, comprises an octane-boosting additive described herein in an amount which is suitable for increasing the octane number of a fuel in a fuel tank or a fuel tanker by at least 0.5, preferably at least 1, and more preferably at least 2, and still more preferably at least 2.5.

Alternatively or additionally, the container, e.g. a container as described previously, comprises an octane-boosting additive described herein in an amount of greater than 100 ml, preferably greater than 150 ml, and more preferably greater than 200 ml. For instance, the octane-boosting additive may be present in the container in an amount of from 300 to 1000 ml, preferably from 350 to 800 ml, and more preferably from 400 to 600 ml. This is believed to be a suitable volume for treating a tank of fuel in a passenger car. Where the octane-boosting additive is used to treat a fuel tanker, e.g. of the type transported on a lorry, the container may comprise an octane-boosting additive described herein in an amount of greater than 5 kg, preferably greater than 10 kg, and more preferably greater than 50 kg.

In another aspect of the invention, a kit comprises a container, e.g. a container as described previously, and instructions for using the octane-boosting additive in a fuel for a spark-ignition internal-combustion engine.

The containers disclosed herein may be manufactured, at least in part and preferably entirely, from metal and/or plastics material. Suitable materials include reinforced thermoplastic materials which for example, may be suitable for storage and use under a range of conditions.

The containers may comprise at least one trade mark, logo, product information, advertising information, other distinguishing feature or combination thereof. The container may be printed and/or labelled with at least one trade mark, logo, product information, advertising information, other distinguishing feature or combination thereof. This may have an advantage of deterring counterfeiting. The container may be of a single colour or multi-coloured. The trademark, logo or other distinguishing feature may be of the same colour and/or material as the rest of the container or a different colour and/or material as the rest of the container. In some examples, the container may be provided with packaging, such as a box or a pallet. In some examples, the packaging may be provided for a plurality of containers, and in some examples a box and/or a pallet may be provided for a plurality of containers.

#### Fuels

The octane-boosting additives and additive compositions described herein may be used in a fuel for a spark-ignition internal combustion engine. It will be appreciated that the octane-boosting additives and additive compositions may be used in engines other than spark-ignition internal combustion engines, provided that the fuel in which the additive or composition is used is suitable for use in a spark-ignition internal combustion engine. Gasoline fuels (including those containing oxygenates) are typically used in spark-ignition internal combustion engines. Commensurately, the fuel composition according to the present invention may be a gasoline fuel composition.

Where the octane-boosting additives described herein are used, e.g. in the form of an additive composition, in a fuel, the resulting fuel composition may comprise a major amount (i.e. greater than 50% by weight) of liquid fuel ("base fuel") and a minor amount (i.e. less than 50% by weight) of octane-boosting additive described herein, i.e. an additive having a chemical structure comprising a 6-membered aromatic ring sharing two adjacent aromatic carbon atoms with a 6- or 7-membered saturated heterocyclic ring, the 6- or 7-membered saturated heterocyclic ring comprising a nitrogen atom directly bonded to one of the shared carbon atoms to form a secondary amine and an atom selected from oxygen or nitrogen directly bonded to the other shared carbon atom, the remaining atoms in the 6- or 7-membered heterocyclic ring being carbon.

Examples of suitable liquid fuels include hydrocarbon fuels, oxygenate fuels and combinations thereof.

Hydrocarbon fuels that may be used in a spark-ignition internal combustion engine may be derived from mineral sources and/or from renewable sources such as biomass (e.g. biomass-to-liquid sources) and/or from gas-to-liquid sources and/or from coal-to-liquid sources.

Oxygenate fuels that may be used in a spark-ignition internal combustion engine contain oxygenate fuel components, such as alcohols and ethers. Suitable alcohols include straight and/or branched chain alkyl alcohols having from 1 to 6 carbon atoms, e.g. methanol, ethanol, n-propanol, n-butanol, isobutanol, tert-butanol. Preferred alcohols include methanol and ethanol. Suitable ethers include ethers having 5 or more carbon atoms, e.g. methyl tert-butyl ether and ethyl tert-butyl ether.

In some preferred embodiments, the fuel composition comprises ethanol, e.g. ethanol complying with EN 15376: 2014. The fuel composition may comprise ethanol in an amount of up to 85%, preferably from 1% to 30%, more preferably from 3% to 20%, and even more preferably from 5% to 15%, by volume. For instance, the fuel may contain ethanol in an amount of about 5% by volume (i.e. an E5

fuel), about 10% by volume (i.e. an E10 fuel) or about 15% by volume (i.e. an E15 fuel). A fuel which is free from ethanol is referred to as an E0 fuel.

Ethanol is believed to improve the solubility of the octane-boosting additives described herein in the fuel. Thus, in some embodiments, for instance where the octane-boosting additive is unsubstituted (e.g. an additive in which R<sub>1</sub>, R<sub>2</sub>, R<sub>3</sub>, R<sub>4</sub>, R<sub>5</sub>, R<sub>6</sub>, R<sub>7</sub>, R<sub>8</sub> and R<sub>9</sub> are hydrogen; X is —O—; and n is 0) it may be preferable to use the additive with a fuel which comprises ethanol.

The fuel composition may meet particular automotive industry standards. For instance, the fuel composition may have a maximum oxygen content of 2.7% by mass. The fuel composition may have maximum amounts of oxygenates as specified in EN 228, e.g. methanol: 3.0% by volume, ethanol: 5.0% by volume, iso-propanol: 10.0% by volume, iso-butyl alcohol: 10.0% by volume, tert-butanol: 7.0% by volume, ethers (e.g. having 5 or more carbon atoms): 10% by volume and other oxygenates (subject to suitable final boiling point): 10.0% by volume.

The fuel composition may have a sulfur content of up to 50.0 ppm by weight, e.g. up to 10.0 ppm by weight.

Examples of suitable fuel compositions include leaded and unleaded fuel compositions. Preferred fuel compositions are unleaded fuel compositions.

In embodiments, the fuel composition meets the requirements of EN 228, e.g. as set out in BS EN 228:2012. In other embodiments, the fuel composition meets the requirements of ASTM D 4814, e.g. as set out in ASTM D 4814-15a. It will be appreciated that the fuel compositions may meet both requirements, and/or other fuel standards.

The fuel composition for a spark-ignition internal combustion engine may exhibit one or more (such as all) of the following, e.g., as defined according to BS EN 228:2012: a minimum research octane number of 95.0, a minimum motor octane number of 85.0 a maximum lead content of 5.0 mg/l, a density of 720.0 to 775.0 kg/m<sup>3</sup>, an oxidation stability of at least 360 minutes, a maximum existent gum content (solvent washed) of 5 mg/100 ml, a class 1 copper strip corrosion (3 h at 50° C.), clear and bright appearance, a maximum olefin content of 18.0% by weight, a maximum aromatics content of 35.0% by weight, and a maximum benzene content of 1.00% by volume.

The fuel composition may contain the octane-boosting additive described herein in an amount of up to 20%, preferably from 0.1% to 10%, and more preferably from 0.2% to 5% weight additive/weight base fuel. Even more preferably, the fuel composition contains the octane-boosting additive in an amount of from 0.25% to 2%, and even more preferably still from 0.3% to 1% weight additive/weight base fuel. It will be appreciated that, when more than one octane-boosting additive described herein is used, these values refer to the total amount of octane-boosting additive described herein in the fuel.

The fuel compositions may comprise at least one other further fuel additive.

Examples of such other additives that may be present in the fuel compositions include those described above as additives which may be present in the additive composition.

Representative typical and more typical independent amounts of additives (if present) and solvent in the fuel composition are given in the table below. For the additives, the concentrations are expressed by weight (of the base fuel) of active additive compounds, i.e. independent of any solvent or diluent. Where more than one additive of each type is present in the fuel composition, the total amount of each type of additive is expressed in the table below.

|    | Fuel Composition                           |                                         |
|----|--------------------------------------------|-----------------------------------------|
|    | Typical amount<br>(ppm, by weight)         | More typical amount<br>(ppm, by weight) |
| 5  | Octane-boosting additives                  | 1000 to 100000                          |
|    | Detergents                                 | 10 to 2000                              |
|    | Friction modifiers and anti-wear additives | 10 to 500                               |
|    | Corrosion inhibitors                       | 0.1 to 100                              |
| 10 | Anti-oxidants                              | 1 to 100                                |
|    | Further octane improvers                   | 0 to 20000                              |
|    | Dehazers and demulsifiers                  | 0.05 to 30                              |
|    | Anti-static agents                         | 0.1 to 5                                |
|    | Other additive components                  | 0 to 500                                |
|    | Solvent                                    | 10 to 3000                              |
| 15 |                                            | 2000 to 50000                           |
|    |                                            | 50 to 300                               |
|    |                                            | 25 to 150                               |
|    |                                            | 0.5 to 40                               |
|    |                                            | 10 to 50                                |
|    |                                            | 50 to 10000                             |
|    |                                            | 0.1 to 10                               |
|    |                                            | 0.5 to 2                                |
|    |                                            | 0 to 200                                |
|    |                                            | 50 to 1000                              |

In some embodiments, the fuel composition comprises or consists of additives and solvents in the typical or more typical amounts recited in the table above

20 Fuel compositions may be produced by a process which comprises combining, in one or more steps, a fuel for a spark-ignition internal combustion engine with an additive composition or octane-boosting additive from a container or a kit of the present invention.

25 In embodiments in which the fuel composition comprises one or more further fuel additives, the further fuel additives may also be combined, in one or more steps, with the fuel.

30 In some embodiments, the additive composition or the octane-boosting additive from a container or kit of the present invention may be combined with the fuel in the form of a refinery additive composition or as a marketing additive composition. Thus, the octane-boosting additive may be combined with one or more other components (e.g. additives and/or solvents) of the fuel composition as a marketing additive, e.g. at a terminal or distribution point. The octane-boosting additive may also be added on its own at a terminal or distribution point from a container or kit of the present invention. The octane-boosting additive may also be combined with one or more other components (e.g. additives and/or solvents such as those described above in connection 35 with the additive composition) of the fuel composition for sale in a container or kit of the present invention, e.g. for addition to fuel at a later time.

40 The octane-boosting additive and any other additives which are to form part of the fuel composition may be incorporated into the fuel composition as one or more additive concentrates and/or additive part packs, optionally comprising solvent or diluent.

45 The additive composition and octane-boosting additive from a container or kit of the present invention may also be added to the fuel within a vehicle in which the fuel is used, either by addition of the composition or additive to the fuel stream or by addition of the composition or additive directly into the combustion chamber.

50 It will also be appreciated that the octane-boosting additive may be added to the fuel, as part of an additive composition, container or kit of the present invention, in the form of a precursor compound which, under the combustion conditions encountered in an engine, breaks down to form an octane-boosting additive as defined herein.

#### Uses and Methods

55 The octane-boosting additives disclosed herein, that form part of an additive composition, container or kit of the present invention, may be used in a fuel for a spark-ignition internal combustion engine. Examples of spark-ignition internal combustion engines include direct injection spark-ignition engines and port fuel injection spark-ignition

13

engines. The spark-ignition internal combustion engine may be used in automotive applications, e.g. in a vehicle such as a passenger car.

Examples of suitable direct injection spark-ignition internal combustion engines include boosted direct injection spark-ignition internal combustion engines, e.g. turbocharged boosted direct injection engines and supercharged boosted direct injection engines. Suitable engines include 5 2.0 L boosted direct injection spark-ignition internal combustion engines. Suitable direct injection engines include those that have side mounted direct injectors and/or centrally mounted direct injectors.

Examples of suitable port fuel injection spark-ignition internal combustion engines include any suitable port fuel injection spark-ignition internal combustion engine including e.g. a BMW 318i engine, a Ford 2.3 L Ranger engine and 10 an MB M111 engine.

The octane-boosting additives disclosed herein may be 20 used, as part of an additive composition or provided by a container or kit of the present invention, to increase the octane number of a fuel for a spark-ignition internal combustion engine. In some embodiments, the octane-boosting additives increase the RON or the MON of the fuel. In 25 preferred embodiments, the octane-boosting additives increase the RON of the fuel, and more preferably the RON and MON of the fuel. The RON and MON of the fuel may be tested according to ASTM D2699-15a and ASTM D2700-13, respectively.

Since the octane-boosting additives described herein increase the octane number of a fuel for a spark-ignition internal combustion engine, they may also be used to address abnormal combustion that may arise as a result of a lower than desirable octane number. Thus, the octane- 30 35 40 45 50 boosting additives described herein, and additive compositions of the present invention which comprise an octane-boosting additive, may be used for improving the auto-ignition characteristics of a fuel, e.g. by reducing the propensity of a fuel for at least one of auto-ignition, pre-ignition, knock, mega-knock and super-knock, when used in a spark-ignition internal combustion engine.

Also contemplated is a method for increasing the octane number of a fuel for a spark-ignition internal combustion engine, as well as a method for improving the auto-ignition 45 50 55 characteristics of a fuel, e.g. by reducing the propensity of a fuel for at least one of auto-ignition, pre-ignition, knock, mega-knock and super-knock, when used in a spark-ignition internal combustion engine. These methods comprise the step of blending an octane-boosting additive or additive composition described herein with the fuel.

The methods described herein may further comprise delivering the blended fuel to a spark-ignition internal combustion engine and/or operating the spark-ignition internal combustion engine.

The invention will now be described with reference to the following non-limiting examples.

## EXAMPLES

60

## Example 1: Preparation of Octane-Boosting Additives

65

The following octane-boosting additives were prepared using standard methods:

14

OX1



OX2



OX3



OX4



OX5



OX6



OX7



OX8



OX9



OX10



**15**

-continued

**16**

-continued

OX11

5

OX12

10

OX13

15

OX14

OX15

25

OX16

30

OX17

35

40

OX18

OX19



Once the octane-boosting additives were prepared, they were introduced into containers comprising means configured to introduce the octane-boosting additive into a fuel system.

**Example 2: Octane Number of Fuels Containing Octane-Boosting Additives**

The effect of octane-boosting additives from Example 1 (OX1, OX2, OX3, OX5, OX6, OX8, OX9, OX12, OX13, OX17 and OX19) on the octane number of two different base fuels for a spark-ignition internal combustion engine was measured.

The additives were added from the containers to the fuels at a relatively low treat rate of 0.67% weight additive/weight base fuel, equivalent to a treat rate of 5 g additive/litre of fuel. The first fuel was an E0 gasoline base fuel. The second fuel was an E10 gasoline base fuel. The RON and MON of the base fuels, as well as the blends of base fuel and octane-boosting additive, were determined according to, ASTM D2699 and ASTM D2700, respectively.

The following table shows the RON and MON of the fuel and the blends of fuel and octane-boosting additive, as well as the change in the RON and MON that was brought about by using the octane-boosting additives:

| Additive | E0 base fuel |      |       |       | E10 base fuel |      |       |       |
|----------|--------------|------|-------|-------|---------------|------|-------|-------|
|          | RON          | MON  | Δ RON | Δ MON | RON           | MON  | Δ RON | Δ MON |
| —        | 95.4         | 86.0 | n/a   | n/a   | 95.4          | 85.2 | n/a   | n/a   |
| OX1      | —            | —    | —     | —     | 97.3          | 86.3 | 1.9   | 1.1   |
| OX2      | 97.7         | 87.7 | 2.3   | 1.7   | 97.8          | 86.5 | 2.4   | 1.3   |
| OX3      | 97.0         | 86.7 | 1.6   | 0.7   | 97.1          | 85.5 | 1.7   | 0.3   |
| OX5      | 97.0         | 86.5 | 1.6   | 0.5   | 97.1          | 85.5 | 1.7   | 0.3   |
| OX6      | 98.0         | 87.7 | 2.6   | 1.7   | 98.0          | 86.8 | 2.6   | 1.6   |
| OX8      | 96.9         | 86.1 | 1.5   | 0.1   | 96.9          | 85.7 | 1.5   | 0.5   |
| OX9      | 97.6         | 86.9 | 2.2   | 0.9   | 97.6          | 86.5 | 2.2   | 1.3   |
| OX12     | 97.4         | 86.3 | 2.0   | 0.3   | 97.3          | 86.1 | 1.9   | 0.9   |
| OX13     | 97.9         | 86.5 | 2.5   | 0.5   | 97.7          | 86.1 | 2.3   | 0.9   |
| OX17     | 97.5         | 86.4 | 2.1   | 0.4   | 97.4          | 86.4 | 2.0   | 1.2   |
| OX19     | 97.4         | 86.1 | 2.0   | 0.1   | 97.6          | 85.9 | 2.2   | 0.7   |

It can be seen that the octane-boosting additives may be used to increase the RON of an ethanol-free and an ethanol-containing fuel for a spark-ignition internal combustion engine.

Further additives from Example 1 (OX4, OX7, OX10, OX11, OX14, OX15, OX16 and OX18) were tested in the E0 gasoline base fuel and the E10 gasoline base fuel. Each of the additives increased the RON of both fuels, aside from OX7 where there was insufficient additive to carry out analysis with the ethanol-containing fuel.

**Example 3: Variation of Octane Number with Octane-Boosting Additive Treat Rate**

The effect of an octane-boosting additive from Example 1 (OX6) on the octane number of three different base fuels for a spark-ignition internal combustion engine was measured over a range of treat rates (% weight additive/weight base fuel).

The first and second fuels were E0 gasoline base fuels. The third fuel was an E10 gasoline base fuel. As before, the RON and MON of the base fuels, as well as the blends of base fuel and octane-boosting additive, were determined according to ASTM D2699 and ASTM D2700, respectively.

The following table shows the RON and MON of the fuels and the blends of fuel and octane-boosting additive, as well as the change in the RON and MON that was brought about by using the octane-boosting additives:

|            | Additive treat rate<br>(% w/w) | Octane number |      |      |      |
|------------|--------------------------------|---------------|------|------|------|
|            |                                | RON           | MON  | ΔRON | ΔMON |
| E0 90 RON  | 0.00                           | 89.9          | 82.8 | 0.0  | 0.0  |
|            | 0.20                           | 91.5          | 83.5 | 1.6  | 0.7  |
|            | 0.30                           | 92.0          | 83.6 | 2.1  | 0.8  |
|            | 0.40                           | 92.5          | 83.8 | 2.6  | 1.0  |
|            | 0.50                           | 92.9          | 83.8 | 3.0  | 1.0  |
|            | 0.67                           | 93.6          | 84.2 | 3.7  | 1.4  |
|            | 1.01                           | 94.7          | 85.0 | 4.8  | 2.2  |
|            | 1.34                           | 95.9          | 85.4 | 6.0  | 2.6  |
|            | 10.00                          | 104.5         | 87.9 | 14.6 | 5.1  |
| E0 95 RON  | 0.00                           | 95.2          | 85.6 | 0.0  | 0.0  |
|            | 0.10                           | 95.9          | 85.8 | 0.7  | 0.2  |
|            | 0.20                           | 96.4          | 86.3 | 1.2  | 0.7  |
|            | 0.30                           | 96.6          | 86.8 | 1.4  | 1.2  |
|            | 0.40                           | 97.1          | 86.6 | 1.9  | 1.0  |
|            | 0.50                           | 97.3          | 87.0 | 2.1  | 1.4  |
|            | 0.60                           | 97.5          | 86.8 | 2.3  | 1.2  |
|            | 0.70                           | 97.8          | 86.8 | 2.6  | 1.2  |
|            | 0.80                           | 98.0          | 87.3 | 2.8  | 1.7  |
|            | 0.90                           | 98.5          | 86.8 | 3.3  | 1.2  |
|            | 1.00                           | 98.7          | 86.9 | 3.5  | 1.3  |
|            | 10.00                          | 105.7         | 88.7 | 10.5 | 3.1  |
| E10 95 RON | 0.00                           | 95.4          | 85.1 | 0.0  | 0.0  |
|            | 0.10                           | 95.9          | 85.2 | 0.5  | 0.1  |
|            | 0.20                           | 96.3          | 86.3 | 0.9  | 1.2  |
|            | 0.30                           | 96.8          | 86.3 | 1.4  | 1.2  |
|            | 0.40                           | 96.9          | 85.8 | 1.5  | 0.7  |
|            | 0.50                           | 97.3          | 85.9 | 1.9  | 0.8  |
|            | 0.60                           | 97.4          | 85.9 | 2.0  | 0.8  |
|            | 0.70                           | 97.9          | 86.0 | 2.5  | 0.9  |
|            | 0.80                           | 98.2          | 86.8 | 2.8  | 1.7  |
|            | 0.90                           | 98.7          | 86.3 | 3.3  | 1.2  |
|            | 1.00                           | 98.8          | 86.5 | 3.4  | 1.4  |
|            | 10.00                          | 105.1         | 87.8 | 9.7  | 2.7  |

Graphs of the effect of the octane-boosting additive on the RON and MON of the three fuels are shown in FIGS. 1a-c. It can be seen that the octane-boosting additive had a significant effect on the octane numbers of each of the fuels, even at very low treat rates.

**Example 4: Comparison of Octane-Boosting Additive with N-Methyl Aniline**

The effect of octane-boosting additives from Example 1 (OX2 and OX6) was compared with the effect of N-methyl aniline on the octane number of two different base fuels for a spark-ignition internal combustion engine over a range of treat rates (% weight additive/weight base fuel).

The first fuel was an E0 gasoline base fuel. The second fuel was an E10 gasoline base fuel. As before, the RON and MON of the base fuels, as well as the blends of base fuel and octane-boosting additive, were determined according to ASTM D2699 and ASTM D2700, respectively.

A graph of the change in octane number of the E0 and E10 fuels against treat rate of N-methyl aniline and an octane-boosting additive (OX6) is shown in FIG. 2a. The treat rates are typical of those used in a fuel. It can be seen from the graph that the performance of the octane-boosting additives described herein is significantly better than that of N-methyl aniline across the treat rates.

A comparison of the effect of two octane-boosting additives (OX2 and OX6) and N-methyl aniline on the octane number of the E0 and E10 fuels at a treat rate of 0.67% w/w is shown in FIGS. 2b and 2c. It can be seen from the graph that the performance of octane-boosting additives described herein is significantly superior to that of N-methyl aniline. Specifically, an improvement of about 35% to about 50% is observed for the RON, and an improvement of about 45% to about 75% is observed for the MON.

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "40 mm" is intended to mean "about 40 mm."

Every document cited herein, including any cross referenced or related patent or application, is hereby incorporated herein by reference in its entirety unless expressly excluded or otherwise limited. The citation of any document is not an admission that it is prior art with respect to any invention disclosed or claimed herein or that it alone, or in any combination with any other reference or references, teaches, suggests or discloses any such invention. Further, to the extent that any meaning or definition of a term in this document conflicts with any meaning or definition of the same term in a document incorporated by reference, the meaning or definition assigned to that term in this document shall govern.

While particular embodiments of the present invention have been illustrated and described, it would be obvious to those skilled in the art that various other changes and modifications can be made without departing from the spirit and scope of the invention. It is therefore intended to cover in the appended claims all such changes and modifications that are within the scope and spirit of this invention.

The invention claimed is:

1. An additive composition comprising an octane-boosting additive and a detergent, wherein the octane-boosting additive has the formula:

19



where:

R<sub>1</sub> is hydrogen;R<sub>2</sub>, R<sub>3</sub>, R<sub>4</sub>, R<sub>5</sub>, R<sub>11</sub> and R<sub>12</sub> are each independently selected from hydrogen, alkyl, alkoxy, alkoxy-alkyl, secondary amine and tertiary amine groups;R<sub>6</sub>, R<sub>7</sub>, R<sub>8</sub> and R<sub>9</sub> are each independently selected from hydrogen, alkyl, alkoxy, alkoxy-alkyl, secondary amine and tertiary amine groups;X is selected from —O— or —NR<sub>10</sub>—, where R<sub>10</sub> is selected from hydrogen and alkyl groups; and

n is 0 or 1;

wherein at least one of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> is selected from a group other than hydrogen.2. An additive composition according to claim 1, wherein R<sub>2</sub>, R<sub>3</sub>, R<sub>4</sub>, R<sub>5</sub>, R<sub>11</sub> and R<sub>12</sub> are each independently selected from hydrogen and alkyl groups.3. An additive composition according to claim 1, wherein R<sub>6</sub>, R<sub>7</sub>, R<sub>8</sub> and R<sub>9</sub> are each independently selected from hydrogen, alkyl and alkoxy groups.4. An additive composition according to claim 1, wherein no more than five of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> are selected from a group other than hydrogen.5. An additive composition according to claim 1, wherein at least one of R<sub>2</sub> and R<sub>3</sub> is hydrogen.6. An additive composition according to claim 1, wherein at least one of R<sub>4</sub>, R<sub>5</sub>, R<sub>7</sub> and R<sub>8</sub> is selected from methyl, ethyl, propyl and butyl groups and the remainder of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> are hydrogen.7. An additive composition according to claim 6, wherein at least one of R<sub>4</sub>, R<sub>5</sub>, R<sub>7</sub> and R<sub>8</sub> is a methyl group and the remainder of R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>11</sub> and R<sub>12</sub> are hydrogen.8. An additive composition according to claim 1, wherein X is —O— or —NR<sub>10</sub>—, where R<sub>10</sub> is selected from hydrogen, methyl, ethyl, propyl and butyl groups.

9. An additive composition according to claim 1, wherein n is 0.

10. An additive composition according to claim 1, wherein the octane-boosting additive is selected from:



20

-continued



11. An additive composition according to claim 1, wherein the octane-boosting additive is present in the additive composition in an amount of at least 10% by weight.

12. A container comprising:

- (i) an octane-boosting additive according to claim 1; and
- (ii) means configured to introduce the octane-boosting additive into a fuel system.

13. A container according to claim 12, wherein the means are configured to couple the container to the fuel system.

14. A container according to claim 12, wherein the means comprise a funnel, a spout, or an injector.

15. A container according to claim 12, wherein the fuel system comprises an engine or a fuel tanker.

16. A container comprising an octane-boosting additive according to claim 1 in an amount which is:

- (a) suitable for treating a fuel in a fuel tank or a fuel tanker at a rate of 0.1% to 10% weight additive/weight base fuel;
- (b) suitable for increasing the octane number of a fuel in a fuel tank or a fuel tanker by at least 0.5; and/or
- (c) greater than 100 ml.

17. A kit comprising:

an octane-boosting additive according to claim 1; and instructions for using the octane-boosting additive in a fuel for a spark-ignition internal-combustion engine.

18. An additive composition comprising an octane-boosting additive and a detergent, wherein the octane-boosting additive is of the formula

US 10,961,477 B2

**21**



5

**22**



10

15

\* \* \* \* \*

or